# EUROPEAN PATENT SPECIFICATION

(11) **EP 3 868 955 B1**
(45) Date of publication and mention of the grant of the patent: **14.06.2023**
(21) Application number: 20158127.9
(22) Date of filing: 19.02.2020
(51) Int. Cl.: E01C 13/08

(54) **ARTIFICIAL TURF HAVING OLIVE PIT PARTICLES**
KUNSTRASEN MIT PARTIKELN VON OLIVENKERNE
GAZON ARTIFICIEL COMPRENANT DES PARTICULES DE NOYAUX D'OLIVES

(43) Date of publication of application: 25.08.2021
(73) Proprietor: FieldTurf, Inc., Montreal QC H4T 1G2 (CA)
(72) Inventor: SMOLLETT, Jason, Montreal, Québec H4T 1G2 (CA); GILL, Darren, Montreal, Québec H4T 1G2 (CA); KRAMER, Tina, Montreal, Québec H4T 1G2 (CA)
(74) Representative: Holme Patent A/S

(56) References cited:
- WO-A2-2014/049531
- US-A1- 2010 055 461
- US-A1- 2018 080 183

## Description

### FIELD OF THE INVENTION

Embodiments of the present invention relate to organic infill systems and artificial turf fields having the same. More particularly, the embodiments relate to organic infill systems comprising olive pit particles and artificial turf fields comprising such infill systems.

### BACKGROUND OF THE INVENTION

There is currently a potential trend and related search with respect to new infill materials and compositions for artificial turf fields. A particular focus has been towards developing an infill that uses organic materials. For example, some customers of infill materials have sought to reduce or eliminate the use of certain compounds such as synthetic materials, recycled rubber, or both for the infill of their artificial turf fields.

As a matter of background, a significant amount of engineering and development is devoted to developing artificial turf field systems. With respect to the infill, each kind of material often times has its own performance and structural characteristics. Obtaining the right composition and arrangement of materials can be challenging.

Examples of prior art can be found in documents US2010/055461A1, US2018/080183A1 and WO2014/049531A2.

### SUMMARY OF THE INVENTION

In accordance with the present invention, there is provided an artificial turf system having the features of claim 1.

Further preferred embodiments are defined by the features of dependent claims 2-7.

### BRIEF DESCRIPTION OF THE DRAWINGS

Various features of examples in accordance with the principles described herein may be more readily understood with reference to the following detailed description taken in conjunction with the accompanying drawings, where like reference numerals designate like structural elements, and in which:
Fig. 1 depicts an illustrative artificial turf system;
Fig. 2 depicts an illustrative artificial turf system in accordance with the present invention;
Fig. 3 depicts yet another illustrative artificial turf system;
Fig. 4 depicts illustrative infill systems in accordance with some embodiments of the present invention;
Fig. 5 depicts the results of an illustrative heat test conducted on the infill systems of Fig. 4 in accordance with some embodiments of the present invention;
Fig. 6 depicts the specific gravity of different materials and the results of an illustrative friction test conducted on those materials in accordance with some embodiments of the present invention;
Fig. 7 depicts the results of an illustrative floatation test conducted on the materials listed in Fig. 6 in accordance with some embodiments of the present invention; and
Fig. 8 depicts the results of an illustrative discoloration test conducted on the materials listed in Fig. 6 in accordance with some embodiments of the present invention.

The components in the figures are not necessarily to scale, emphasis instead being placed upon illustrating the principles of the invention. Moreover, all illustrations are intended to convey concepts, where relative sizes, shapes and other detailed attributes may be illustrated schematically rather than literally or precisely.

### DETAIL DESCRIPTION OF THE INVENTION

In this specification, the following non-SI unit is used, which may be converted to the respective SI or metric unit according to the following conversion table:
Feet convert to centimeters : 1 foot = 30,48 cm.

In accordance with principles of the present invention, embodiments of the present invention are directed to using olive pit particles as a portion or a primary portion of the infill for an artificial turf field. Infill 105, as shown in Figs. 1-3, refers to material that is deposited over the turf backing 120 and forms a layer around the turf fibers 125. Infill 105 is interspersed between the turf fibers 125 rising out of the turf backing 120. Infill 105 generally has a depth that covers a portion of the turf fibers 125 (unexposed portion of the turf fiber) leaving part of the turf fibers 125 extending above the infill 105 (exposed portion of the turf fiber). Infill 105 helps support the turf fibers 125 in an upright position and is used to provide traction and shock absorption.

The turf fibers 125 are preferably synthetic fibers or man-made fibers. The turf fibers 125 can be made of materials comprising polyethylene ("PE"), polypropylene ("PP"), polyamide ("PA"), other types of polymers, or a combination thereof. The fibers 125 can be monofilament fibers, slit film fibers, fibrillated fibers, texturized fibers, or a combination thereof. In some embodiments, however, naturally occurring fibers, grass, vegetation, or plants may also be used, either alone or in combination with the synthetic fibers. The turf backing 120 can be made of woven or non-woven sheet material and one or more of sheets of such material. The turf backing 120 can be porous or permeable to provide water drainage. Woven or non-woven sheet material may be polypropylene, polyesters, or other synthetic materials. The pile height H of the artificial turf should have a measurement between about 15 mm and about 70 mm. The pile height H refers to the distance measured from the bottom surface of the turf backing 120 (the surface to be contacted by the ground or other installation surface) to the tip of the fibers 125. Other heights of the fibers and pile are also contemplated depending on the height of the infill and thickness of the turf backing. The fibers 125 can be attached to the turf backing 120 by tufting, weaving (pile weave, flat weave, etc.), knitting, needle punching, fusion bonding and flocking, heating, pressurizing, adhering (e.g., using adhesive or other binder), or a combination thereof. The fibers 125 and the backing 120 can be held together only at the locations where they contact, e.g., applying adhesive to only locations where they are tufted, creating rows of adhesive and the areas in between are without adhesive. The system formed by the infill 105, turf backing 120, and fibers 125 may be referred to as the artificial turf system 100. The artificial turf system 100 may further include a pad that is positioned under the turf backing 120 to provide additional shock absorption. An artificial turf field comprises one or more artificial turf systems 100.

The infill 105 has a height G between about 2 mm and about 30 mm and a weight between about 1 kg per square meter and about 15 kg per square meter of olive pit particles. In other words, in a square meter of infill, the total weight of olive pit particles in that area is between about 1 kg per square meter and about 15 kg per square meter. The infill 105 may contain olive pit particles only (e.g., Fig. 1) or a combination of olive pit particles and other infill materials such as sand (e.g., Figs. 2-3), whether they are intermixed or deposited in separate layers. In the former case (olive pit particles only), the total weight of the infill equals the total weight of the olive pit particles, which is about 1 kg per square meter and about 15 kg per square meter. In the latter case (combination), the total weight of the infill is different or larger than the total weight of the olive pit particles. For example, the total weight of the infill 105 may be between about 3 kg per square meter and about 21 kg per square meter, if the total weight of the olive pit particles is between about 1 kg per square meter and about 15 kg per square meter and the total weight of the other infill material is between about 2 kg per square meter and about 6 kg per square meter. Other heights and weights of the infill and/or olive pit particles are also contemplated depending on the height of the fibers and thickness of the turf backing.

In one embodiment, the infill 105 comprises at least one layer of particles comprising olive pit particles (e.g., Figs. 2-3). The olive pit particles include olive pit particles that have a sieve size of between 8 and 50 (0.3 mm - 2.36 mm), or preferably between 10 and 35 (0.5 mm - 2.0 mm). The olive pit particles that have a sieve size of between 8 and 50, or preferably between 10 and 35, are at least 1% by weight of the olive pit particles. Preferably, the olive pit particles of such sieve sizes are at least 1% and no more than 10% by weight of the olive pit particles (or between about 1% and about 10%). More preferably, the olive pit particles of such sieve sizes are at least 1% and no more than 5% by weight of the olive pit particles (or between about 1 % and about 5%).

The olive pit particles described in this application are preferably raw or untreated crushed olive pits. For example, the preferred olive pit particles are naturally occurring olive pit particles or such particles that have not been treated with antimicrobial additives (whether it is chemical, artificial, organic, natural, non-toxic, or non-irritating antimicrobial additives). Antimicrobial additives may be agents used to prevent the growth of bacteria, fungi, mold, or other microorganisms and animals (e.g., to prevent decomposition, contamination, etc.), and/or to strengthen the mechanical properties of the materials or components being treated (e.g., can withstand larger amount of ultraviolet, larger amount of friction before they breaks, etc.). In some embodiments, the other layers or materials and components (e.g., turf fibers, turf backing, and infill) of the artificial turf system are also not treated with antimicrobial additives. In some embodiments, the infill, whether internally or externally, is not treated with antimicrobial additives. Olive pit particles are particles produced by applying mechanical force to raw or naturally occurring olive pits to break or crush the pits into smaller pieces of particles (e.g., using a grinder, granulator, or cracker mill). In some embodiments, raw or untreated olive pits (not crushed) may also be used. Olive pit and olive stone are used interchangeably in this application to refer to the same component. An olive pit or olive stone refers to a seed of an olive before it is crushed or an uncrushed seed. Olive pit particles refer to particles resulting from crushing the pit, stone, or seed. The olive pit particles, infill systems, or artificial turf systems are used or implemented without water or adding water to the particles or systems. The olive pit particles, infill systems, or artificial turf systems are dry, either completely dry (e.g., 0% of water, vapor, or moisture) or dry enough such that the amount of water, vapor, or moisture in these particles or systems are negligible or cannot be sensed or felt when a person with ordinary skill in the art touches the particles or systems. Water-retaining particles, either particles containing only water or partially water (e.g., a percentage of water and another percentage of a different liquid, solid, or other material) are also not necessary (e.g., not added into the infill or artificial turf system or not used in crushing the olive pits).

In some embodiments, the infill may comprise extruded composite (e.g., thermoplastic elastomer (TPE), thermoplastic rubbers, mineral composite, or a combination thereof), cork, rubber (e.g., Styrene-butadiene rubber or SBR, or Ethylene Propylene Diene Monomer rubber or EPDM rubber), other organic materials, or a combination thereof. Mineral composite preferably includes carbonate mineral, carbonite mineral, or both. The different materials may be used as separated layers in the infill or intermixed to form the infill (one intermixed layer that makes up the entire infill). The infill may be prepared with or without rubber. When the infill is prepared without rubber, the infill is devoid of rubber, crumb rubber, rubber materials, or other similar materials (collectively referred to as rubber materials). The olive pit particles are used to replace rubber materials. Infill that is substantially devoid rubber materials) is also contemplated. For example, 65% or higher or 75% or higher by weight of the infill is not rubber materials. Infill that is primarily devoid of rubber materials is also contemplated. For example, 50% or higher by weight of the infill is not rubber materials. Rubber materials or the layer comprising rubber materials is directed to provide shock absorption. Depending on the amount of rubber materials used, these materials or layer may be substantially, primarily, or the only materials or layer that provides the function of shock absorption. The olive pit particles based on the aforementioned sieve sizes and weight percentages may also be used in combination with the materials stated in this paragraph (either intermixed or use as separate layers).

The infill materials and compositions described in this application have been tested and compared to other organic infills and compositions. The test results show that the described infill materials and compositions have significant better heat reduction capability compared to other organic infills and compositions. Such infill materials and compositions and improvement were not previously found and do not exist in artificial turf technology. The improvement is attributed to at least the described infill materials, compositions, or both. The improvement and/or the described infill materials and compositions that exhibit such property were not known to or expected by a person with ordinary skill in the art in the field of artificial turf and related fields until the embodiments of the present invention are developed. It should be noted the heat reduction characteristic is an improvement in addition to meeting or exceeding the required sports performance (such as the required ball bounce, ball roll, amount of vertical compression in response to applied force, and amount of shock absorption in EN 15330-1, EN 12235, EN 12234, EN 14808, EN14809, and other standards and methods) and exhibiting other properties.

Fig. 4 depicts several illustrative infills, infill compositions, or infill systems that are used in a heat test. The infill systems used in the test include a cork-based infill system, a first olive stone-based infill system (olive pits-based infill system), a first extruded composite-based infill system, a second extruded composite-based infill system, and a second olive stone-based infill system. The cork-based infill system and the first olive stone-based infill system are dual layers or dual materials system and their pictorial illustrations are shown in Fig. 2. Each of the cork-based infill system and the first olive stone-based infill system includes a stabilizing infill (first layer or material) 110 and a performance infill (second layer or material) 115. The stabilizing infill 110 includes sand only or primarily sand and the performance infill 115 includes olive stones (olive pits) only or primarily olive stones.

The other infill systems are triple layers or triple materials systems and their pictorial illustrations are shown in Fig. 3. These systems further include a mixed layer 130 (third layer or material) of sand and rubber only, or a mixed layer 130 of primarily sand and rubber. The mix layer 130 may be an intermixed layer of sand and rubber, or a layer of sand and another layer of rubber. Preferably, the rubber is rubber particles having a sieve size of between 14 and 30 (0.6 mm - 1.4 mm). The first extruded composite-based infill system includes a first performance infill and the second extruded composite-based infill system includes a second performance infill. Each of the performance infills includes extruded composite infill and is referred to first extruded composite infill and second extruded composite infill. The first extruded composite infill includes a first amount of TPE and a first amount of carbonate mineral or carbonite mineral, and the second extruded composite infill include a second amount of TPE and a second amount of carbonate mineral or carbonite mineral. The first extruded composite infill and the second extruded composite infill differ in at least one of these amounts. The first and second extruded composite infills (and the stabilizing infill and mix layer) do not contain any olive pits or olive pit-based materials.

In the infill systems shown in Fig. 4, the performance infill is preferable the layer that is exposed to foot traffic. Therefore, in an artificial turf with the dual layer system, the artificial turf includes a backing layer, the stabilizing infill layer on top of (overlaying) the backing layer, and the performance infill layer on top of (overlaying) the stabilizing infill layer. In an artificial turf with the triple layer system, the artificial turf includes a backing layer, the stabilizing infill layer on top of the backing layer, the mix layer on top of the stabilizing infill layer, and the performance infill layer on top of the mix layer. The backing layer is the layer that contacts or is closer to the ground or an installation surface. It is understood all these infill systems may include additional layers or materials, be arranged in a different order, or have the described layers or materials substituted. The layers or materials in the infill system may also be intermixed and used as one layer. Other combinations are also possible. For convenience, the present description primarily focuses on two and three layer infill systems.

Fig. 4 also shows the weight of each infill material or layer in the infill system. For example, referring to the second olive stone-based infill system, the sand of the stabilizing infill is about 5 kg per square meter, the olive stones of the performance infill is about 2 kg per square meter, the sand of the mix layer is about 25 kg per square meter, and the rubber of the mix layer is about 12.5 kg per square meter.

Fig. 5 depicts the results of a heat test conducted on the infill systems show in Fig. 4. The same heat test is conducted (the same test setup is used) on each infill system. In each setup, the temperature of each infill system is measured from the same location, such as determined by a (X,Y,Z) coordinate like the center of the infill system. For example, in an infill system having a length of 2 feet, a width of 2 feet, and a depth of 2 feet ((2, 2, 2,)), the center point is a location where the length is 1 foot, the width is 1 foot, and the depth is 1 foot ((1,1,1)).

The results show that the olive stone-based infill systems based on the composition described in this application exhibit a lower temperature than the other organic infill systems after exposing to the same heat source or extreme temperature for the same period of time. After two hours, the temperature measured from the same location in the olive stone-based infill systems are 58°C and 59°C. In contrast, the temperature measured from the same location in the other organic infill systems are 63°C, 66°C, and 72°C. After four hours, the temperature measured from the same location in the olive stone-based infill systems are 61°C and 62°C. In contrast, the temperature measured from the same location in the other organic infill systems are 65°C, 69°C, and 62°C. Moreover, within the first several minutes (e.g., 10 minutes, 15 minutes) of the test, the olive stone-based infill systems also show a slower function or rate in reaching their highest or stable temperature from their initial temperature.

Tests over 4 hours long also have been conducted (e.g., days and weeks) and they all show that the olive stone-based infill systems based on the composition described in this application always exhibit a lower temperature and a slower heat absorbing function than the other organic infill systems. Tests also have been repeated and measured from other locations (e.g., (1, 0.75, 1.5) location from each infill system) and the same trends or characteristics also have been observed.

The olive stone-based infill systems based on the composition described in this application have a superior heat reduction or radiating capability than the other organic infill systems in Fig. 4 and other existing organic infill systems. A superior heat reduction or radiating capability keeps an artificial turf cooler (and thus keeps the overall sports field or stadium cooler to the players and audience), reduces heat damage to the tufted fibers, minimizes burning sensation to human skin when athletes fall, makes the artificial turf less susceptible to fire, allows the organic particles and other particles to degrade slower, and curtail other heat-related issues.

Fig. 6 depicts the specific gravity of three different types of organic materials (olive, cork, and coconut particles) and the result of the friction tests conducted on those materials. Olive particles have a specific gravity greater than 1 to prevent floating and below 1.5 to meet certain sports requirements. The tests are performed by a friction equipment that simulates the fall and sliding of an athlete on the surface of these materials by measuring the temperature of these materials, or the temperature elevation or burn felt by an athlete. The temperature also indicates or can be used to determine the amount of friction felt by the athlete (e.g., with the shoes, skin, or clothes). In the tests, conditions imitating athlete weights from 25 kg to 150 kg and falling or sliding speed up to 5 meter per second had been used on the materials in Fig. 6 (or artificial turf systems with such materials). The result shows the average temperatures of the conducted friction tests. The results shows that the olive pits have a lower temperature compared to that of cork. Although coconut particles also exhibit a low temperature, they require water or need to be wetted in order to achieve that temperature (e.g., either 50% of the total coconut particles by weight had been soaked in water before they are tested or an amount of water equal to 50% of the total coconut particle weight had been added to the coconut particles.) This complicates the installation and preparation processes of an infill system and may make the artificial turf system incompatible with certain sports or disqualify the artificial turf system from meeting certain standards (EN 15330-1, EN 12235, etc.).

Fig. 7 depicts the result of a floatation test conducted on the olive, cork, and coconut particles. Each glassware is filled with about the same amount of olive, cork, and coconut particles (e.g., the total weight of the particles is about the same) and then about the same amount of water is poured into each glassware. After letting the combination sits for approximately 30 minutes, the test shows that the olive particles stay in the bottom of the glassware (do not float in the water) whereas the cork and coconut particles float on or toward the surface of the water. This shows that the olive particles are more stable than the cork and coconut particles when they are filled with water or their infill systems are filled water. The olive particles are more likely to stay in place on rainy days and are more difficult to be dislodged from the artificial turf. Therefore, olive pit particles infill system is a better option in maintaining the structure and look of the infill system and keeping an even surface when water is involved (e.g., olive particles are less likely to be moved from place to place).

Fig. 8 depicts the result of a discoloration test conducted on the olive, cork, and coconut particles. The discoloration test is conducted by placing olive, cork, and coconut particles in their respective containers with water and immersing or mixing the particles with water for several hours (e.g. about 2 hours). A new, white piece of clothes (e.g., made of cotton, polyester, nylon, or a combination thereof) is then dipped in each of the containers to absorb water therein and removed from the respective container. The test shows that the olive particles leave behind the lightest color or almost no color on its respective clothes compared to those of the cork and coconut particles. The coconut particles leave behind the darkest color. Therefore, the olive pit particles are more preferable and would make shirts, shorts, or other wears on the athletes less dirty, such as when they fall or slide.

In any of the above embodiments, the illustrative weight percentages can mean approximate weight percent ages, instead of exact weight percentages. The term approximate or about means ±0.5%, preferably ±0.2%, and more preferably ±0.1 % of the illustrative weight percentage. For example, approximate or about 5% by weight means between and including 4.9% and 5.1 % by weight. Exemplary infills and artificial turf systems are described for illustrative purposes. Further, since numerous modifications and changes will readily be apparent to those having ordinary skill in the art, it is not desired to limit the invention to the exact constructions as demonstrated in this disclosure. Accordingly, all suitable modifications and equivalents may be resorted to falling within the scope of the invention. Applications of the technology to other fields are also contemplated.

## Claims

1. An artificial turf system (100) having a pile height (H) between about 15 mm and about 70 mm and comprising:
a turf backing layer (120),
a plurality of turf fibers (125) attached to the turf backing layer (120), and
a dual layers infill (105), the first layer of said infill (105) being a stabilizing infill layer (110) on top of the turf backing layer (120) and overlaying said turf backing layer (120),
the second layer of said infill (105) being a performance infill layer (115) on top of the stabilizing infill layer (110) and overlaying the stabilizing infill layer (110),
wherein said infill (105) is interspersed between the turf fibers (125) supporting the turf fibers (125) in an upright position and having a depth covering a portion of the turf fibers (125) and exposing another portion of the turf fibers (125), wherein the infill (105) comprises olive pit particles and another infill material,
wherein the performance infill layer (115) is an olive pit particles layer having a weight between about 1 kg per square meter and about 15 kg per square meter of olive pit particles, and the stabilizing infill layer (110) is a layer of said another infill material being sand.

2. The system of claim 1, wherein the olive pit particles are raw crushed olive pits.

3. The system (100) of claim 1, wherein the infill (105) is untreated with antimicrobial additives.

4. The system (100) of claim 1, wherein the infill (105) has a height between about 2 mm and about 30 mm.

5. The system (100) of claim 1, wherein the infill (105) has a weight between about 1 kg per square meter and about 15 kg per square meter of olive pit particles.

6. The system (100) of claim 1, wherein the system comprises 22 kg per square meter of sand and 13 kg per square meter of olive pit particles.

7. The system (100) of claim 1, wherein the plurality of turf fibers (125) are attached to the turf backing layer (120) by tufting, weaving, such as pile weave or flat weave, knitting, needle punching, fusion bonding and flocking, heating, pressurizing, adhering, such as adhering using adhesive or other binder.

## Patentansprüche

1. Kunstrasensystem (100) mit einer Stapelhöhe (H) zwischen etwa 15 mm und etwa 70 mm und umfassend:
eine Rasenträgerschicht (120),
eine Mehrzahl von Rasenfasern (125), die an der Rasenträgerschicht (120) befestigt sind, und
eine doppellagige Füllung (105),
wobei die erste Lage der Füllung (105) eine stabilisierende Füllungslage (110) auf der Rasenträgerschicht (120) ist und die Rasenträgerschicht (120) überlagert,
wobei die zweite Lage der Füllung (105) eine Leistungsfüllungslage (115) auf der stabilisierenden Füllungslage (110) ist und die stabilisierende Füllungslage (110) überlagert,
wobei die Füllung (105) zwischen den Rasenfasern (125) verteilt ist, die die Rasenfasern (125) in einer aufrechten Position tragen und eine Tiefe aufweisen, die einen Teil der Rasenfasern (125) bedeckt und einen anderen Teil der Rasenfasern (125) freilegt, wobei die Füllung (105) Olivengrubenpartikel und ein anderes Füllungsmaterial umfasst,
wobei die Leistungsfüllungslage (115) eine Olivenkernpartikellage mit einem Gewicht zwischen etwa 1 kg pro Quadratmeter und etwa 15 kg pro Quadratmeter Olivenkernpartikel ist und die stabilisierende Füllungslage (110) eine Lage eines anderen Füllungsmaterials ist, das Sand ist.

2. System nach Anspruch 1, wobei die Olivenkernpartikel rohe zerkleinerte Olivenkerne sind.

3. System (100) nach Anspruch 1, wobei die Füllung (105) nicht mit antimikrobiellen Zusatzstoffen behandelt ist.

4. System (100) nach Anspruch 1, wobei die Füllung (105) eine Höhe zwischen etwa 2 mm und etwa 30 mm aufweist.

5. System (100) nach Anspruch 1, wobei die Füllung (105) ein Gewicht zwischen etwa 1 kg pro Quadratmeter und etwa 15 kg pro Quadratmeter Olivenkernpartikel aufweist.

6. System (100) nach Anspruch 1, wobei das System 22 kg pro Quadratmeter Sand und 13 kg pro Quadratmeter Olivenkernpartikel umfasst.

7. System (100) nach Anspruch 1, wobei die Mehrzahl von Rasenfasern (125) an der Trägerschicht (120) durch Tufting, Weben, wie etwa Florbindung oder Flachbindung, Stricken, Nadelstanzen, Schmelzbinden und Beflocken, Erwärmen, Druckbeaufschlagen, Kleben, wie etwa Kleben unter Verwendung von Klebstoff oder einem anderen Bindemittel, befestigt sind.

## Revendications

1. Un système de gazon synthétique (100) qui possède une hauteur de brin (H) entre environ 15 mm et environ 70 mm et qui comprend :
une couche de support de gazon (120) ;
plusieurs fibres de gazon (125) qui sont fixées à la couche de support de gazon (120) ; et
un remplissage (105) sous la forme d'une double couche, la première couche dudit remplissage (105) représentant une couche de remplissage de stabilisation (110) qui est disposée par-dessus la couche de support de gazon (120) et qui recouvre ladite couche de support de gazon (120), la seconde couche dudit remplissage (105) représentant une couche de remplissage de performance (115) qui est disposée par-dessus la couche de remplissage de stabilisation (110) et qui recouvre ladite couche de remplissage de stabilisation (110);
dans lequel ledit remplissage (105) est intercalé entre les fibres de gazon (125) en supportant les fibres de gazon (120) dans une position verticale et possède une profondeur qui recouvre une portion des fibres de gazon (125) et qui expose une autre portion des fibres de gazon (125); dans lequel le remplissage (105) comprend des particules de noyaux d'olives et une autre matière de remplissage ;
dans lequel la couche de remplissage de performance (115) représente une couche de particules de noyaux d'olives dont le poids se situe entre environ 1 kg par mètre carré et environ 15 kg par mètre carré de particules de noyaux d'olives, et la couche de remplissage de stabilisation (110) représente une couche de ladite autre matière de remplissage, à savoir du sable.

2. Le système selon la revendication 1, dans lequel les particules de noyaux d'olives représentent des noyaux d'olives grossièrement broyés.

3. Le système (100) selon la revendication 1, dans lequel le remplissage (105) n'est pas traité avec des additifs antimicrobiens.

4. Le système (100) selon la revendication 1, dans lequel le remplissage (105) possède une hauteur entre environ 2 mm et environ 30 mm.

5. Le système (100) selon la revendication 1, dans lequel le remplissage (105) possède un poids entre environ 1 kg par mètre carré et environ 15 kg par mètre carré de particules de noyaux d'olives.

6. Le système (100) selon la revendication 1, dans lequel le système comprend 22 kg par mètre carré de sable et 13 kg par mètre carré de particules de noyaux d'olives.

7. Le système (100) selon la revendication 1, dans lequel lesdites plusieurs fibres de gazon (125) sont fixées à la couche de support de gazon (120) par touffetage, par tissage sous la forme d'une armure velours ou d'une armure toile, par tricotage, par aiguillage, via une liaison par fusion et par flocage, par chauffage, par compression, par adhérence, par exemple par adhérence en utilisant un adhésif ou un autre liant.
